



US007516605B2

(12) **United States Patent**  
**Goldwater et al.**

(10) **Patent No.:** **US 7,516,605 B2**  
(45) **Date of Patent:** **Apr. 14, 2009**

(54) **ELECTRONIC ELONGATION-SENSING  
ROPE**

(75) Inventors: **Dan Goldwater**, Emeryville, CA (US);  
**Saul Griffith**, Emeryville, CA (US);  
**Eric Wilhelm**, Oakland, CA (US); **Colin  
Bulthaup**, Oakland, CA (US)

(73) Assignee: **Makani Power, Inc.**, Alameda, CA (US)

(\*) Notice: Subject to any disclaimer, the term of this  
patent is extended or adjusted under 35  
U.S.C. 154(b) by 672 days.

(21) Appl. No.: **11/074,292**

(22) Filed: **Mar. 7, 2005**

(65) **Prior Publication Data**

US 2005/0231207 A1 Oct. 20, 2005

**Related U.S. Application Data**

(60) Provisional application No. 60/521,200, filed on Mar.  
10, 2004.

(51) **Int. Cl.**

**D02G 3/02** (2006.01)  
**D02G 3/22** (2006.01)

(52) **U.S. Cl.** ..... **57/238; 57/264**

(58) **Field of Classification Search** ..... **57/264,  
57/265**

See application file for complete search history.

(56) **References Cited**

**U.S. PATENT DOCUMENTS**

|                |         |                        |          |
|----------------|---------|------------------------|----------|
| 5,182,779 A *  | 1/1993  | D'Agostino et al. .... | 385/13   |
| 5,834,942 A *  | 11/1998 | De Angelis .....       | 324/522  |
| 6,276,215 B1 * | 8/2001  | Berg .....             | 73/800   |
| 6,361,299 B1 * | 3/2002  | Quigley et al. ....    | 428/35.9 |
| 7,117,981 B2 * | 10/2006 | Logan et al. ....      | 187/391  |
| 7,123,030 B2 * | 10/2006 | Robar et al. ....      | 324/693  |
| 7,326,139 B2 * | 2/2008  | Eichhorn et al. ....   | 474/260  |

\* cited by examiner

*Primary Examiner*—Shaun R Hurley

(74) *Attorney, Agent, or Firm*—Van Pelt, Yi & James LLP

(57) **ABSTRACT**

A fibrous tension member comprises a plurality of structural threads and an indicator thread. The indicator thread modulates one or more electrical properties of the indicator thread based at least in part on the elongation of the indicator thread. A system for sensing elongation of a fibrous tension member comprises a plurality of structural threads, at least one indicator thread, and a sensing-processing device. The sensing-processing device is electrically connected to the at least one indicator thread to determine the elongation of the fibrous tension member.

**8 Claims, 20 Drawing Sheets**





Fig. 1



Fig. 2



Fig. 3



Fig. 4



Fig. 5



Fig. 6



Fig. 7



Fig. 8



Fig. 9



Fig. 10



Fig. 11



Fig. 12



Fig. 13



Fig. 14



Fig. 15



Fig. 16a



Fig. 16b



Fig. 17



Fig. 18



Fig. 19



Fig. 20

**1**  
**ELECTRONIC ELONGATION-SENSING  
ROPE**

**CROSS-REFERENCE TO RELATED  
APPLICATIONS**

This non-provisional patent application claims priority benefit of U.S. provisional patent application No. 60/521,200 filed on Mar. 10, 2004, the disclosure of which is expressly incorporated herein in its entirety by reference.

**STATEMENT REGARDING FEDERALLY  
SPONSORED RESEARCH**

Not Applicable

**REFERENCE TO MICROFICHE APPENDIX**

Not Applicable

**FIELD OF THE INVENTION**

The present invention relates to systems and methods for measuring elongation or curvature experienced globally or locally by an elongate fibrous tension member.

**BACKGROUND OF THE INVENTION**

Almost any type of material which can be twisted, pulled, extruded, spun, stretched, or otherwise fabricated into a filament or fiber can be used to make ropes. Basically, a rope is an elongate structural element which is fabricated from any collection of elongated members, such as filaments or fibers, which are manufactured into some type of a long, structural line which is relatively flexible and capable of carrying tensile loads.

Herein, the term "rope" refers to rope, cord, wire rope, cable, and the like.

Herein, the term "webbing" refers to fibrous tension members which are substantially flat and comprised of fibers woven, bundled, knit, braided, felted, or twisted together. Webbing includes strong, narrow, closely woven fabric used especially for seat belts and harnesses or in upholstery.

Herein, the term "fibrous tension member" refers to rope or webbing comprising multiple threads woven, bundled, knit, braided, felted, or twisted-together such that the resultant member is at least somewhat flexible.

Elongation, stress, and strain are generally related to each other. For example, if a rope supporting a load elongates one inch and is operating in its elastic range, the strain is also one inch and the stress may be deduced by knowing the length of rope being loaded, its spring constant, and knowing whether elongation is increasing or decreasing (hysteresis). If one tracks elongation over time, one knows which hysteresis curve should be used to relate elongation to stress. Also, if one tracks elongation over time, one can distinguish non-recoverable plastic deformation (yield) from elastic strain. For these reasons, for the purposes of this application in both the specification and the claims, the term "elongation" refers to elongation, stress, or strain.

Most common ropes are manufactured by the following process:

1. Relatively short to moderately long filaments or fibers are twisted into yarns.
2. Yarns are twisted into cords.
3. Cords are twisted into strands. This process is called "forming." Sometimes, extra cords, yarns, and/or fila-

**2**

ments (made from relatively flexible materials) are added during the forming process for internal lubrication in each strand. These extra cords, yarns, and/or filaments are commonly used during the fabrication of ropes that are subjected to relatively high flexural loads.

- 5 4. Two or more strands are twisted into a rope. This process is called "laying." Similar to Step 3, extra strands, cords, yarns, and/or filaments (made from relatively flexible materials) can be added during the laying process to improve internal lubrication in the rope.
- 10 5. Two or more ropes are twisted into a wire rope or cable. Similar to Step 4, extra elongated members can be added to improve internal lubrication in the cable.

Ropes may alternatively be manufactured using bundling, weaving, and/or felting techniques. Many ropes have external materials applied to the yarns, cords, or strands to improve environmental resistance, as well as handling characteristics. Application processes for these materials include galvanizing, bonding, painting, and coating.

- 15 20 Ropes and webbing are integral to a wide range of activities. The potential cost in equipment damage, personnel injuries and even lives of failing or overloaded ropes is high. The fiscal cost of maintaining and inspecting ropes and webbing is high. Safety factors in ropes and webbing are significant, on order five to fifteen times expected load, with inherent weight cost.
- 25

An external load sensing element such as a load cell can be used to measure stress on a rope. This provides stress measurement at a point such as a pulley connection or the interface between the rope and a load. However, sometimes the elongation varies along the rope which would not be discernable with a point measurement such as that provided by a load cell. In addition, some applications such as rock climbing, would not easily allow the permanent connection of a load cell to a rope so the rope may be used when it is not monitored, allowing damage to occur without monitoring.

- 30 35 40 Various means have been proposed for providing an indication of damage to ropes and webs. In U.S. Pat. No. 5,834,942 to Pethrick et. al., a synthetic fiber cable is disclosed which includes one or more electrically conductive indicator threads placed into the strands to monitor the state of the cable. A tearing of the fiber may be detected by applying a voltage to the indicator thread. In this manner, each individual strand of a synthetic fiber cable can be checked and the cable can be replaced when a predetermined number of torn strands have been exceeded.

In the case of the above-mentioned patent, the indicator threads and sensing unit are capable of detecting when a threshold voltage limit value is exceeded by torn indicator threads. The Pethrick system particularly shows a threshold value switch SW to binarize the output and their discussion speaks only of setting this threshold value to that which would indicate breakage of the indicator thread.

- 45 50 55 In the case of the above-mentioned patent, the indicator threads connect to the sensing unit via connecting elements—physical contacts at the end of the cable. This limits the application to cases where the end of the cable is accessible to the sensing unit and the data produced refers to the cable's entire length as there is no provision for sensing a portion of the cable.

Various means have been proposed for providing a measure of strains and kinks in ropes. In U.S. Pat. No. 5,182,779 to D'Agostino et al., a rope is disclosed which includes one or more optical fibers placed into the strands to monitor the state of the rope. Such a system is capable of measuring strain in the rope by means of detecting Rayleigh reflections due to density fluctuations. Such a system can detect macrobends

and microbends which change the angle at which light strikes the interface between core and clad, causing light to be absorbed into the clad or reflected back to the source. Such a system can use optical time domain reflectometry (OTDR) to detect and locate breaks resulting in Fresnel reflections. Such a system can use preformed optical fiber to minimize residual stresses in the indicator fiber resulting from twisting in the rope manufacturing process. Preforming is the process of twisting an elongated member, such as a filament in the opposite direction as the twisting process to make a rope so the indicator thread is relatively untwisted in the final rope. Such a system can use prestressed rope to allow the rope to strain past the breaking point of the optical indicator fiber.

Such a system requires a sophisticated optical sensing-processing unit. Accordingly, there is a need in the art for an improved system and method for measuring elongation or curvature experienced globally or locally by fibrous tension members.

#### SUMMARY OF THE INVENTION

The present invention provides an a fibrous tension member such as rope or webbing having means for electrical sensing of elongation which solves at least some of the above-noted problems. The applicants have developed and tested prototypes of a new class of multi-functional rope structure where the incorporation of metallic or conducting fibers in the proper configurations and fiber placements (known as rope constructions) leads to ropes and cables that can electronically sense their loading condition and/or continuously record their loading history. In accordance with one aspect of the present invention, a fibrous tension member comprises, in combination, at least one indicator thread. The indicator thread comprises discrete segments of conductive fibers. The indicator thread also comprises means for electrical sensing of elongation of the fibrous tension member.

According to another aspect of the present invention, a method for sensing elongation of a tension member comprising the steps of, in combination, providing a fibrous tension member with at least one indicator thread and providing the indicator threads with discrete segments of conductive fibers. A sensing-processing device is electrically connected to the indicator thread to determine the elongation of the tension member.

From the foregoing disclosure and the following more detailed description of various preferred embodiments it will be apparent to those skilled in the art that the present invention provides a significant advance in the technology and art of electronic elongation-sensing rope. Particularly significant in this regard is the potential the invention affords for providing a high quality, durable, reliable, versatile, and relatively inexpensive system. Additional features and advantages of various preferred embodiments will be better understood in view of the detailed description provided below.

#### BRIEF DESCRIPTION OF THE DRAWINGS

These and further features of the present invention will be apparent with reference to the following description and drawings, wherein:

FIG. 1 shows an indicator thread comprising a "whipped" (i.e. helically-wrapped) bare conductive fiber interleaved with whipped non-conductive fiber;

FIG. 2 shows an indicator thread comprising a whipped insulated conductive fiber.

FIG. 3 shows an indicator thread comprising a whipped conductive fiber with an inductively coupled sensor attached to outside of rope;

FIG. 4 shows a rope with a pair of electrically resistive indicator fibers connected to each other at one end of the rope, allowing sensing from the other end of the rope where a connector allowing direct connection to an external sensor is mounted;

FIG. 5 shows an indicator thread comprising a coaxial indicator thread connected to a sensing device;

FIG. 6 shows an indicator thread comprising discrete conductive and discrete non-conductive fibers;

FIG. 7 shows an indicator thread comprising discrete conductive and continuous non-conductive fibers;

FIG. 8 shows an indicator thread which changes in conductivity along its length;

FIG. 9 shows a coaxial indicator thread which changes in capacitance along its length;

FIG. 10 shows a coaxial indicator thread which changes in inductance along its length;

FIG. 11 shows a rope with multiple indicator threads configured to allow sensing device to locate which region of the rope is experiencing the sensed elongation;

FIG. 12 shows a situation where, due to winching, one might want to measure the elongation of a rope in just a section of the rope;

FIG. 13 shows a rope with two indicator threads on opposite sides of a kink in the rope. Their differential elongation allows the sensing device to measure curvature in the rope;

FIG. 14 shows an indicator thread with multiple direct-connect tap points along its length;

FIG. 15 shows a rope with an indicator fiber with periodic whipped sections allowing a sensing device to inductively couple to the indicator thread at these inductive tap points;

FIG. 16a shows a rope with three indicator threads each with direct-connect tap points staggered both along and around the periphery of the rope;

FIG. 16b shows the same rope in section;

FIG. 17 shows an indicator thread with multiple direct-connect tap points along its length connected to a sensing device;

FIG. 18 shows a rope with three indicator threads each with direct-connect tap points staggered around the periphery of the rope connected to a sensing device;

FIG. 19 shows rope with two indicator fibers, a sensing device attached to one, and an external splice allowing the sensing device to measure characteristics of the rope section between the sensed endpoint and the splice; and

FIG. 20 shows a rope with indicator thread and an embedded sensor which wirelessly transmits elongation data to an external receiver.

It should be understood that the appended drawings are not necessarily to scale, presenting a somewhat simplified representation of various preferred features illustrative of the basic principles of the invention. The specific design features of fibrous tension members as disclosed herein, including, for example, specific dimensions, orientations, and shapes will be determined in part by the particular intended application and use environment. Certain features of the illustrated embodiments have been enlarged or distorted relative to others to facilitate visualization and clear understanding. In particular, thin features may be thickened, for example, for clarity or illustration. All references to direction and position, unless otherwise indicated, refer to the orientation of the fibrous tension members illustrated in the drawings.

The following reference numbers are used in the specification and drawings:

|     |                                                                  |
|-----|------------------------------------------------------------------|
| 10  | indicator bundle                                                 |
| 11  | indicator thread                                                 |
| 12  | core                                                             |
| 13  | non-conductive thread                                            |
| 20  | indicator bundle                                                 |
| 21  | helically-wrapped indicator thread                               |
| 22  | core                                                             |
| 23  | test equipment                                                   |
| 30  | whipped indicator thread                                         |
| 31  | inductive pickup                                                 |
| 32  | test equipment                                                   |
| 40  | rope-end jumper                                                  |
| 41  | rope-end terminal                                                |
| 50  | coax indicator bundle                                            |
| 51  | core conductor                                                   |
| 52  | insulator                                                        |
| 53  | sheath conductor                                                 |
| 54  | test equipment for coax                                          |
| 60  | rope                                                             |
| 61  | structural thread                                                |
| 62  | indicator thread                                                 |
| 63  | discrete conductive fiber                                        |
| 64  | discrete non-conductive fiber                                    |
| 65  | rope sheath                                                      |
| 66  | test equipment                                                   |
| 67  | test equipment lead                                              |
| 70  | indicator thread                                                 |
| 71  | discrete conductive fiber                                        |
| 72  | continuous non-conductive fiber                                  |
| 80  | indicator thread with high resistance per unit length            |
| 81  | indicator thread with low resistance per unit length             |
| 82  | rope with changing resistance indicator thread                   |
| 90  | coax with changing capacitance                                   |
| 91  | region of low capacitance per unit length                        |
| 92  | region of high capacitance per unit length                       |
| 93  | dielectric                                                       |
| 94  | core                                                             |
| 100 | whipped indicator bundle with changing inductance                |
| 101 | indicator thread                                                 |
| 102 | region of low inductance per unit length                         |
| 103 | region of high inductance per unit length                        |
| 104 | core                                                             |
| 110 | rope with three indicator cable to localize elongation           |
| 111 | test equipment to localize elongation                            |
| 113 | region of low conductivity for thread 116                        |
| 114 | region of low conductivity for thread 117                        |
| 115 | region of low conductivity for thread 118                        |
| 116 | indicator thread with one region of low conductivity             |
| 117 | indicator thread with one region of low conductivity             |
| 118 | indicator thread with one region of low conductivity             |
| 120 | rope being winched onto a spool                                  |
| 121 | load suspended by a rope                                         |
| 122 | spool                                                            |
| 123 | test equipment connecting to adjacent tap points                 |
| 124 | tap points on rope                                               |
| 130 | indicator thread on outside of the kink                          |
| 131 | indicator thread on inside of the kink                           |
| 132 | test equipment to measure differential elongation                |
| 140 | rope with tap points along                                       |
| 141 | indicator fiber in core of rope                                  |
| 142 | tap point                                                        |
| 150 | indicator bundle                                                 |
| 151 | whipped sections of indicator thread                             |
| 152 | straight sections of indicator thread                            |
| 153 | inductively-coupling test equipment                              |
| 160 | rope with three indicator threads                                |
| 161 | indicator thread traveling in rope core                          |
| 162 | tap point where indicator thread emerges from core               |
| 170 | sensing device to measure between adjacent tap points            |
| 180 | ring connector                                                   |
| 181 | connector terminal                                               |
| 182 | test equipment for connecting to multiple tap points around rope |
| 190 | jumper                                                           |
| 191 | tap points                                                       |
| 192 | test equipment                                                   |
| 193 | indicator threads                                                |

-continued

|   |     |                                            |
|---|-----|--------------------------------------------|
| 5 | 194 | rope                                       |
|   | 200 | indicator thread                           |
|   | 201 | wireless transmitting sensor-processor     |
|   | 202 | wireless data receiver                     |
|   | 203 | rope with embedded wireless test equipment |

## 10 DETAILED DESCRIPTION OF CERTAIN PREFERRED EMBODIMENTS

15 It will be apparent to those skilled in the art, that is, to those who have knowledge or experience in this area of technology, that many uses and design variations are possible for the fibrous tension members disclosed herein. The following detailed discussion of various alternative and preferred embodiments will illustrate the general principles of the invention with reference to specific embodiments. Other 20 embodiments suitable for other applications will be apparent to those skilled in the art given the benefit of this disclosure.

### Discrete Segments

25 A preferred embodiment of the present invention is illustrated in FIG. 6. In this system, the fibrous tension member is a rope 60. The rope 60 consists of a sheath 65 encapsulating seven threads consisting of six structural threads 61 and one indicator thread 62. The front two structural threads 61 are removed in the drawing to show the indicator thread 62 in the core of the rope 60. The electrical indicator thread 62 consists of 30 80% by weight non-conductive polyester fibers 64 chosen for their structural strength and 20% by weight discrete segments of conductive stainless steel fibers 63. The length and diameter of the conductive fibers 63 affects the electrical characteristics of the indicator thread. We have found that 35 conductive fibers with diameters 5-10  $\mu$ m and lengths 5-50 mm have provided good response. As a tensile load is applied axially to the rope 60, the conductive 63 and non-conductive 64 fibers are compressed transaxially, increasing the surface contact of adjacent conductive fibers 63 and decreasing the overall resistance of the indicator thread 62. As the tension is 40 further increased, the conductive fibers 63 are stretched, reducing their cross-section and increasing their resistance. The resistivity of the indicator thread 62 is modulated by these effects, and that modulation can be tailored by the choice of the construction method of the rope 60 by, for 45 example, controlling the proportion of conductive fibers 63, properties of the non-conductive fibers 64 and how conductive fibers 63 are mixed in, the length, diameter, or composition of conductive fibers 63, and the placement of indicator thread 62 in the rope 60.

50 In some embodiments, discrete segments have an average length of less than 100,000 times their diameter. In some embodiments, an indicator thread (e.g., indicator thread 72) 55 comprises between 0.25% and 50% of conducting fiber by volume. In some embodiments, an indicator thread (e.g., indicator thread 72) comprises between 1% and 60% of conducting fiber by weight. In some embodiments, an indicator thread is configured to provide elongation sensing along a 60 length exceeding 100 times an average diameter of the fibrous tension member. As shown in FIG. 7, the indicator thread 72 may consist of continuous non-conductive fibers 70 instead of discrete. The conductive fibers 71 remain discrete to reduce sensitivity of system to strain-induced conductive fiber 71 65 breakage.

Fibrous tension members are commonly made from a hierarchy of threads. Larger threads are composed of smaller

threads, larger strands are composed of smaller strands. The preferred embodiment of the invention may include hierarchical composition of the fibrous tension member, and may include hierarchical composition of the indicator thread.

#### Loop to Make Circuit

In order to measure the resistance of an indicator thread, it must form a complete circuit with the test equipment. As shown in FIG. 6, the test equipment 66 may be connected via test equipment leads 67 to the indicator thread 62 at each end of the rope 60. Alternatively, as shown in FIG. 4, two indicator threads 62 pass through the rope 60 and are attached via a rope-end jumper 40 at one end and rope end terminals 41 connected to the test equipment 66 to form a closed circuit with regard to the test equipment 66. Alternatively, a single conductive fiber can be run through the rope and serve as the 'ground' for all other indicator threads. At the end of the rope all indicator threads are connected to the ground wire. This ground conductor may be made with a lower resistance than the indicator threads so it does not much influence the resistivity of the indicator thread measurements. The system may be configured so that the test equipment 66 provides enough power to the indicator thread 62 to warm it. This may be used to maintain pliability of the fibrous tension member in cold weather.

#### Kink Detection

For many rope applications it is useful to know if a rope is kinked. As shown in FIG. 13, this can be detected by running two indicator threads 130 & 131 down opposite sides of the outer surface of the rope 60. If the rope 60 is kinked, the indicator thread on the outside of the kink 130 will be highly strained, while the indicator threads on the inside of the kink 131 will be relaxed. The test equipment to measure differential elongation 132 can then monitor the difference in strain between the indicator threads 130 & 131. If the rope 60 is strained linearly (pulled in a straight direction) then both indicator threads 130 & 131 will increase in resistance equally, but if the rope 60 is kinked then the indicator threads 130 & 131 will change resistance relative to each other. Typically, one would use at least three indicator threads in order to detect curvature in any axis. For improved accuracy and redundancy more than three indicator threads can be used.

#### Interface—Integrated

A small microcontroller and battery can be integrated directly into the end of the rope to read out the status of the indicator threads. The microcontroller can be turned on by pressing or squeezing an actuator which is on or within the rope and the data can be displayed to a small LCD or LED display, a patch of electrochromic material or via an audio transducer. This would be useful for climbing ropes or other applications where one wants to periodically check the status of the rope, but not necessarily in real time.

#### Interface—External

For applications with many different ropes that need to be periodically inspected a small portable readout device could be built that would have a microcontroller with rechargeable battery and a more sophisticated display. The device would clamp onto the rope at a region where the indicator threads are on the surface of the rope and accessible to the device. The data from the indicator threads can be read out in real-time, logged, and alarms can be programmed to go off if measured characteristics of indicator threads in the rope fall outside an acceptable range.

#### Interface—Wireless

For larger more permanent ropes, as shown in FIG. 20, a sensing-processing device 201 can be integrated into the rope 203, coupled to the indicator fiber 200, and powered by a long lifetime battery or wired to a power source. The sensing-

processing device 201 could communicate its data in real-time over a wireless network such as bluetooth or 802.11. The data from many different ropes could all be collected by a central server 202, analyzed, and presented to the user.

#### 5 Tap Points Along

If the rope incorporates several indicator threads it may be necessary to make electrical connections to each of the individual indicator threads to read out the data. As shown in FIG. 14, one way to do this is to run each of the indicator threads 10 141 on the inside of the rope 140 and then periodically bring each indicator thread to the outside of the rope 140 as a tap point 142 for a short length of the rope. These tap points 142 may be color-coded so that they are easy to identify and make connections to.

15 As shown in FIG. 17, the user attaches a sensing device 170 to the outside of the rope 140 and it can make a direct electrical connection to two adjacent tap points 142. This is useful as shown in FIG. 12, where a sensed rope 120 with tap points 124 along its length is being winched onto a spool 122. The 20 elongation of the rope 120 on the spool 122 may not be the same as the elongation of the rope 120 off the spool 122 and close to the load 121 hanging from the rope 120. A test equipment 123 is shown making direct connection to adjacent tap points 124 on the rope 120 allowing elongation in that 25 section of the rope 120 to be measured.

30 Alternatively, as shown in FIG. 15, the indicator bundle 150 may have periodic sections where the indicator thread is highly whipped 151 interleaved with sections where the indicator thread is less whipped 152. A test equipment 153 may be inductively coupled to this pair of inductive tap points 151. Note that although the test equipment 153 is shown coupling to the indicator bundle 150 from one side, effectively coupling to the whipped sections of the indicator thread 151 is 35 likely to require the test equipment to encircle the indicator bundle 150.

Conductive tap-points can be constructed during or after the braiding process by causing an indicator thread from the 40 core to be brought to the sheath and then returned to the core over a short length span. Tap-points could also be created by adding an extra conductive element to the rope during or after the braiding process which connects the desired indicator thread to the outside of the rope.

45 Herein, the term "tap point" refers to sections of a fibrous tension member providing electrical connectivity to an external sensing-processing unit by means of direct electrical contact or coupling to an electromagnetic field.

#### Tap Points Around

50 Alternatively, as shown in FIGS. 16a (the rope shown along its length) & 16b (the rope shown in axial section at a tap point junction), all the indicator threads may travel in the core 161 for some length of the rope 160 and then emerge to the periphery of the rope 160 as a set of tap points 162 spaced periodically around its circumference. As shown in FIG. 18, a 55 ring connector 180 composed of periodically spaced connector terminals 181 could be attached around the rope 160 to simultaneously connect all the tap points to the test equipment 182. In order to distinguish between the indicator threads, the tap points may be arranged with a non-symmetry such as by omitting one indicator thread. This would key the 60 rope and allow the test equipment to identify which indicator thread is which.

As shown in FIG. 19, a jumper 190 may be applied to a pair (or more) of tap points 191. This allows the test equipment 192 to sense the indicator threads 193 between the end of the 65 rope 194 and the jumpered 190 tap points 191. This is an easy non-permanent way to make a loop. It allows making a loop at any pair of tap points using a simple clamp-on device.

## Whipped—Inductively Measured

FIG. 6 shows the indicator threads 62 oriented substantially parallel to the rope 60 axis. The shown indicator thread 62 may be replaced with an indicator bundle 20 as shown in FIG. 2. Here, the indicator bundle 20 consists of an indicator thread 21 “whipped” (i.e. helically-wrapped) around a core 22, forming a coil. The indicator thread 21 may be bare or insulated and is composed of discrete segments of conductive fibers. The core 22 may be conductive or non-conductive.

Voltage along a whipped indicator thread 21 is proportional to rate of change of current supplied by the test equipment 23 and the coil’s 21 coefficient of self inductance. Said coefficient is a purely geometric quantity, having to do with the sizes, shapes, and relative orientations of the loops of the indicator thread 21. As the helix is strained axially, the mutual inductance of the loops decreases as does the measured inductance of the indicator thread 21.

As shown in FIG. 1, the indicator bundle 10 may employ a bare indicator thread 11 helically-wrapped around a core 12 where adjacent coils of the indicator thread 11 are insulated from each other by interlacing a whipped non-conductive thread 13.

## Whipped—Inductive Coupling to Sensor

As shown in FIG. 3, voltage may be induced in a whipped indicator thread 30 by the electromagnetic interaction with an inductive sensing device 31. The induced voltage is a function of the mutual inductance between the whipped indicator thread 30 and the inductive pickup 31 which is itself connected to a test equipment 32. The mutual inductance is in part a function of the whipped indicator’s size, shape and orientation of coil loops. As the whipped indicator’s helix is elongated axially, the mutual inductance decreases.

## Coax

As shown in FIG. 5, the indicator bundle 50 may be configured as a coaxial cable. An indicator thread 51 (which is itself composed of discrete conductive fibers as in FIG. 6), is sheathed in insulation 52 which is itself surrounded by a conductive sheath 53. This conductive sheath 53 may be a sheet material, continuous conductive fibers running parallel to the bundle axis, woven S- and Z-oriented wires as typically used in coaxial cable construction, or a whipped thread (as shown in FIG. 2). A connected test equipment 54 measures capacitance or transmission line properties via standard means such as time domain reflectrometry (TDR), frequency domain reflectometry (FDR) or spectrum analysis. Some test methods may require an electrical termination device to be connected from the indicator thread 51 to the conductive sheath 53 at the end of the coaxial cable.

## Preforming and Prestressing

Depending on the fibrous tension member fabrication and elongation sensing methods, the indicator threads may be preformed to reduce or eliminate residual stresses which are created during the yarn making process. Preforming is the process of twisting an elongated member, such as a filament (or the like) in the opposite direction as the twisting process to make a cord, yarn, strand so that the elongated member is relatively untwisted in the manufactured cord, yarn, or strand.

## Sampling Rate

Loads may be applied to the fibrous tension member axially, radially, torsionally, or in combination. Indicator threads may be incorporated into the fibrous tension member in appropriate number and position to optimally measure desired information of expected loads. Loads may be static, random, or periodic with respect to time. If it is desired to characterize random or periodic loads, the Nyquist criterion will determine sampling rate requirements. This criterion

states that if a waveform is to be reconstructed after sampling, that waveform must be sampled at twice the fundamental frequency.

## Indicator Thread with Changing Resistance

As shown in FIG. 8, a resistance-sensed conductive indicator thread 80 & 81 (of the type shown in FIG. 6) incorporated into a rope 82 may change in conductivity along its length. For example, the indicator thread may have a section with high resistance per unit length 80 surrounded by sections with low resistance per unit length 81.

## Indicator Thread with Changing Capacitance

As shown in FIG. 9, a capacitance-sensed conductive indicator bundle 90 incorporated into a rope may change in capacitance along its length. For example, the indicator bundle may have a section with low capacitance per unit length 91 surrounded by sections with high capacitance per unit length 92. Capacitance per unit length is a function of the area and distance between the conductive core 94 and the conductive sheath 92. Capacitance per unit length is also a function of the dielectric 93 insulating these two electrodes.

## Indicator Thread with Changing Inductance

As shown in FIG. 10, an inductance-sensed indicator bundle 100 incorporated into a rope may change in inductance along its length. In this example, the indicator thread 101 is helically wrapped with changing pitch around a non-conductive core 104. The indicator bundle 100 has a section with low inductance per unit length 102 surrounded by sections with high inductance per unit length 103. This configuration is more sensitive to elongation in the tightly coiled areas 103. The change in inductance per length due to elongation of the loosely coiled section 102 is less than that of the tightly coiled section 103.

## Independently Measuring Elongation in Multiple Rope Segments

FIG. 11 shows how a rope 110 with three indicator threads 116, 117, 118 are used to measure elongation in three different regions 113, 114, 115, respectively, of the rope 110. This could be useful if elongation is non-uniform along the length of the rope 110 and the application requires understanding the elongation gradient along the rope 110. Alternatively, in the case of winching a rope onto a spool, the length of rope 110 subject to the stress of a load changes as more or less rope 110 is played out off the spool. This requires that the measured characteristics of the rope 110 are calibrated against the length of rope 110 experiencing that load. FIG. 11 shows how a rope 110 can deliver elongation data for sections of rope 113, 114, 115 to test equipment 111 where each section has identical length. Indicator thread 116 has lower conductivity in region 113 and higher conductivity in regions 114 and 115.

This makes it more sensitive to elongation in region 113. Similarly, indicator thread 117 has lower conductivity in region 114 and higher conductivity in regions 113 and 115. This makes it more sensitive to elongation in region 114.

In general, “N” separate indicator threads will provide “N” independent elongation measurements using resistive measurement. Capacitive or inductive-sensed indicator threads/bundles can be used instead of the shown resistive-sensed indicator threads 116, 117, 118. Indicator bundles sensed with transmission line analysis can provide richer information about elongation along the thread.

From the foregoing detailed description, it can be appreciated that the illustrated fibrous tension members provide a new ‘intelligent textile’ product category that enables fibrous tension members to signal their own elongation electronically to a sensing-processing unit which may be external or incorporated into the fibrous tension member. The present invention uses electrical indicator threads to measure elongation

## 11

rather than simple breaks. The present invention also allows the sensing device to connect to the fibrous tension member at a variety of locations along the fibrous tension member. When desired, the present invention further allows the sensing device to measure elongation for a region of the fibrous tension member instead of along the entire length of the fibrous tension member.

From the foregoing detailed description, it can also be appreciated that the illustrated fibrous tension members provide the following advantages:

1. Overall or localized electronic sensing of elongation in fibrous tension members;
2. Overall or localized electronic sensing of curvature such as kinks in fibrous tension members;
3. Overall or localized self-heating of fibrous tension members for cold climate applications;
4. Convenient interface between fibrous tension member and sensing-processing device by means of direct connection tap points around periphery or along length of fibrous tension member;
5. Convenient interface between fibrous tension member and sensing-processing device by means of non-contact inductive coupling; and
6. Incorporation of sensing-processing device into the fibrous tension member to ensure that all elongations are recorded and means to communicate acquired data via direct connection or wirelessly.

As an example of the potential use for this technology, consider recreational climbing ropes which are rated to be used up to a yield strain. The addition of an intelligent sensor would remove the risk and uncertainty of trying to estimate how much a rope has been strained. In addition, many ropes are supposed to be retired after they have strained past a certain critical point a certain number of times. An intelligent system could monitor and keep track of how many times the rope has been critically strained.

As an additional example, electric cables such as high tension power lines: these could be enhanced by adding a thin intelligent rope sheathing around the outside of the cable. This intelligent rope material could inform the power company when it is under unusual tension, such as when a tree branch falls on the cable. This would allow the cable owners to perform preventative maintenance on the cable, thus averting outages.

From the foregoing disclosure and detailed description of certain preferred embodiments, it will be apparent that various modifications, additions and other alternative embodiments are possible without departing from the true scope and spirit of the present invention. The embodiments discussed were chosen and described to provide the best illustration of the principles of the present invention and its practical application to thereby enable one of ordinary skill in the art to utilize the invention in various embodiments and with various modifications as are suited to the particular use contemplated. All such modifications and variations are within the scope of the present invention as determined by the appended claims when interpreted in accordance with the benefit to which they are fairly, legally, and equitably entitled.

What is claimed is:

1. The fibrous tension member comprising:  
a plurality of structural threads; and  
an indicator thread, wherein the indicator thread indicates elongation by modulating one or more electrical properties based at least in part on the elongation of the fibrous tension member, and wherein the indicator thread changes one or more electrical properties along its length, and wherein said indicator thread includes at

## 12

least two portions and one of the two portions is substantially more conductive per unit length than the other of the two portions.

2. The fibrous tension member, comprising:  
a plurality of structural threads; and  
an indicator thread, wherein the indicator thread indicates elongation by modulating one or more electrical properties based at least in part on the elongation of the fibrous tension member, and wherein the indicator thread changes one or more electrical properties along its length, and wherein said indicator thread includes at least two portions and one of the two portions is substantially more inductive per unit length than the other of the two portions.
3. The fibrous tension member, comprising:  
a plurality of structural threads; and  
an indicator thread, wherein the indicator thread indicates elongation by modulating one or more electrical properties based at least in part on the elongation of the fibrous tension member, and wherein the indicator thread changes one or more electrical properties along its length, and wherein said indicator thread includes at least two portions and one of the two portions is substantially more electrically capacitive per unit length than the other of the two portions.
4. The fibrous tension member, comprising:  
a plurality of structural threads; and  
an indicator thread, wherein the indicator thread indicates elongation by modulating one or more electrical properties based at least in part on the elongation of the fibrous tension member, and wherein the indicator thread changes one or more electrical properties along its length, and wherein the fibrous tension member comprises at least two of said indicator threads with dissimilar electrical response properties in a section of the fibrous tension member.
5. The fibrous tension member of claim 4, further comprising means for distinguishing elongation in said section from elongation response elsewhere along said fibrous tension member.
6. The fibrous tension member, comprising:  
a plurality of structural threads; and  
an indicator thread, wherein the indicator thread indicates elongation by modulating one or more electrical properties based at least in part on the elongation of the fibrous tension member, and wherein the fibrous tension member comprises at least two of the indicator threads and the two indicator threads extend along a common segment of the fibrous tension member, the two are electrically insulated from each other along a length of said segment, the two indicator threads are electrically connected together at one end of the segment, and the two indicator threads are configured to connect to a sensing-processing interface device at the other end of the segment to form a circuit.
7. A method for sensing elongation of a fibrous tension member comprising:  
providing a fibrous tension member a plurality of structural threads;  
providing a fibrous tension member at least one indicator thread, wherein the at least one indicator thread indicates elongation by modulating one or more electrical properties based at least in part on the elongation of the fibrous tension member;  
electrically connecting a sensing-processing device to the at least one indicator thread to determine the elongation of the fibrous tension member.

**13**

8. A system for sensing elongation of a fibrous tension member comprising:

a fibrous tension member comprising a plurality of structural threads;

a fibrous tension member comprising at least one indicator thread, wherein the at least one indicator thread indicates elongation by modulating one or more electrical prop-

5

**14**

erties based at least in part on the elongation of the fibrous tension member; and

a sensing-processing device, wherein the sensing-processing device is electrically connected to the at least one indicator thread to determine the elongation of the fibrous tension member.

\* \* \* \* \*

UNITED STATES PATENT AND TRADEMARK OFFICE  
**CERTIFICATE OF CORRECTION**

PATENT NO. : 7,516,605 B2  
APPLICATION NO. : 11/074292  
DATED : April 14, 2009  
INVENTOR(S) : Goldwater et al.

Page 1 of 1

It is certified that error appears in the above-identified patent and that said Letters Patent is hereby corrected as shown below:

**Claim 1**

Column 11, line 60 delete “member comprising:” and insert -- member, comprising: --

**Claim 5**

Column 12, line 37 delete “claim 4,further” and insert -- claim 4, further --

Signed and Sealed this

Twenty-second Day of September, 2009



David J. Kappos  
*Director of the United States Patent and Trademark Office*